

Oct. 22, 1963

MASATOMO KUSUNOSE ETAL

3,107,970

PROCESS FOR THE MANUFACTURE OF HIGH TENACITY VISCOSE RAYON

Filed Sept. 28, 1961



## 1

3,107,970

### PROCESS FOR THE MANUFACTURE OF HIGH TENACITY VISCOSE RAYON

Masatomo Kusunose, Yasuo Saji, and Takeo Koyasu, all of Itano-gun, Tokushima, Japan, assignors to Toho Rayon Kabushiki Kaisha, Tokyo, Japan, a corporation of Japan

Filed Sept. 28, 1961, Ser. No. 141,356  
Claims priority, application Japan Oct. 4, 1960  
4 Claims. (Cl. 18—54)

The present invention relates to a process for the manufacture of viscose rayon, which comprises heating unaged viscose to a temperature above that of a spinning bath, extruding the thus heated viscose in a low temperature acidic sulfate bath containing formaldehyde, and stretching the resulting threads in a second bath, namely in a double bath stretching method.

It is an object of this invention to provide regenerated viscose fibers capable of supplying fabrics of high tenacity, high resistance to alkali and excellent dimensional stability, in other words, to provide viscose rayon of high tensile strength, high dry and wet strength and good resistance to alkali and high resistance to swelling.

Referring to the spinning of viscose to such a regenerated viscose fiber, particularly when an excellent regenerated fiber is sought which is appropriate for a certain specific purpose, it has usually been well-known to attain a close relationship between respective properties of the particular viscose and a suitable coagulating and regenerating method that is very well suitable for each property of the viscose.

According to this invention, a type of viscose sufficiently removed of so-called "structure" is shaped to filaments by an extremely slow regeneration and then by imparting resulting filaments crystallization and arrangement effects substantially simultaneously to impart the regenerated fiber a highly crystalline property and orientation.

In view of the above relationship, the substance of the present invention is based on a knowledge that an excellent fiber of a high wet tensile strength can be obtained by heating a relatively insufficiently aged viscose at high temperatures to decompose so-called "structure" for improving dispersion property and regenerating by introducing thus treated viscose into a spinning bath which contains formaldehyde and is kept at a temperature lower than that of the viscose at least by 20° C.

Technical elements for this invention lie in close combination of the use of viscose heated at high temperatures with the use of spinning bath containing formaldehyde and being held at a temperature lower than that of the viscose at least by 20° C. The effect is remarkably high especially in cases viscose of a relatively high polymerization degree is treated, and regenerated fibers of excellent properties can be obtained.

The quantity of carbon bisulfide required for the manufacture of viscose in the practice of this invention ranges from 35 to 55% of the amount of cellulose used and, in addition, no particularly high  $\gamma$ -value is required.

The required alkali content of the viscose is in a range of 0.5 to 0.9 times its content of cellulose, and a departure from such a range results in degradation of the product obtained.

In particular, when low alkaline viscose is used which

## 2

contains low alkali less than 0.5 times the content of cellulose, the dispersion of cellulose molecules in the viscose is unfavorable. Accordingly, a good result as referred to later can not be obtained because the function of formaldehyde contained will then be disturbed.

Moreover, unaged viscose of a salt index above 9 must be used. Furthermore, when the ripening is in progress, the quality of products lowers. With progress of ripening the structure develops unfavorably to the practice of this invention similarly as described before.

High viscosity viscose, which viscosity varies from 50 to 400 seconds and preferably higher than 100 seconds, should be used. From viscose of a viscosity below 50 seconds a fragile product of a poor knot strength can only be obtained.

According to the present invention, viscose is used after it has been heated from 45° to 70° C. and a range from 55° to 66° C. is optimum. Various apparatus and methods are used for heating viscose. It is necessary to heat the viscose rapidly and uniformly as much as possible near the spinneret.

Generally, viscose is heated by providing a heat exchanger whose heat source is heated water in the neighborhood of the spinneret. Such heated viscose should be spun in a spinning bath of a temperature held at least 20° C. below that of the viscose. In this case, the thus heated viscose is kept from being cooled by the low temperature of the spinning bath at a part of the viscose pipe immediately before the spinneret immersed in the spinning bath.

The spinning bath according to this invention is 35° C. maximum bath containing from 50 to 150 gm./liter  $\text{Na}_2\text{SO}_4$ , from 1 to 10 gm./liter formaldehyde, 30 gm./liter max.  $\text{ZnSO}_4$  and 40 gm./liter min.  $\text{H}_2\text{SO}_4$ .

In the present process wherein formaldehyde is added to such a relatively low temperature spinning bath, operational obstruction due to stimulous smell of formaldehyde can be alleviated remarkably.

Attempts of raising polymerization degrees of cellulose molecules constituting regenerated fibers have long been made to improve the quality of products. In order to accomplish above purpose, decrease of the cellulose concentration in the viscose is avoided, which in turn requires necessarily to spin high viscosity viscose.

Thus, a number of specific spinning processes for high viscosity viscose have been introduced.

According to this invention, in which a viscose of such high viscosity as ranging from 50 to 400 seconds is spun under specific conditions necessary for this invention, no excellent property fiber anticipated by this invention may be obtained by merely adding formaldehyde to the spinning bath. On the contrary, in many instances the quality of the product is lowered. The viscose is considered to require to receive the action of a spinning bath which contains formaldehyde in the state of so-called decomposed structure as described before.

Principal functions of formaldehyde added to the spinning bath are considered to disturb the coagulation and formation of nuclei for OH radicals due to hydrogen bond or others of regenerated cellulose of filaments coming out from the spinning bath.

Since viscose is stretched in this unrestrained condition of OH-radicals in the second high temperature bath, it is considered possible to provide enough high tension and

develop highly crystalline structure and simultaneously attain a high degree of orientation.

Particularly when the viscosity of viscose increases, mutual constraining of cellulose molecules in the viscose becomes high and the viscose includes much "structure."

When such viscose as just referred to enters in a relatively low temperature spinning bath and is subject to reaction of formaldehyde, the constraint received by the molecules in the viscose is considered to act in such a way that the action of formaldehyde may be disturbed. Therefore, in order to enable a relatively low temperature spinning of a high viscosity viscose and obtain in addition an effective action of formaldehyde, it is required to increase the temperature of the viscose at the spout of the spinning bath as compared with the temperature of said bath.

When the temperature of the spinning bath is not within the above-mentioned range, the spinning operation lacks smoothness to lower the quality of products. When the concentration of  $\text{Na}_2\text{SO}_4$  is less than 50 gm./liter, variation in concentration due to  $\text{Na}_2\text{SO}_4$  which occurs in the spinning bath is high and the process control and preparation of the spinning bath become difficult.

The essential requirement for the present invention is heating viscose in such a way that the temperature of the viscose entering the spinning bath may be at least 20° C. higher than that of the spinning bath and moreover above 40° C. When the viscose is spun in an ordinary process, a remarkably inferior quality product can only be obtained as compared with the case with the present invention.

The present invention is carried out according to the double bath stretching spinning process and if necessary a third or a higher number of baths may be used.

The most remarkable feature of the regenerated cellulose fiber obtained in this invention is a high wet modulus. This is numerically compared by tension (gm.) per denier required for 5% elongation on the load-elongation curve (FIGURE 1) when wet.

TABLE 1

Load required for 5% extension  
when wet gm./denier

|                                    |           |
|------------------------------------|-----------|
| Product of the present invention   | Above 1.5 |
| Ordinary viscose rayon             | 0.20      |
| Usual high strength staple fiber A | 0.20      |
| Usual high strength staple fiber B | 0.70      |
| Usual high strength staple fiber C | 0.90      |
| Usual high strength staple fiber D | 1.25      |

As the result of a further investigation on the process of this invention, the strength of the fiber manufactured by the process as described above has been found to be dependent on the stretch condition after spinning.

Considering first over the stretching condition for spun filaments vs. strength of fibers obtained, the present inventor has made various experiments on the effect of the rates of stretching or elongations (percent) X, Y and Z upon the strength of the threads obtained. If the velocity of filaments being reeled on the first spool from the first bath is  $a$  m./min.; that of the filaments being reeled on the second spool after passing through the second bath (i.e. the first stretching bath) is  $b$  m./min.; and that of the filaments being reeled on the third spool after passing through the third bath (i.e. the second stretching bath) is  $c$  m./min., the elongation X (percent) in the first stretching bath is:

$$X = \left( \frac{b}{a} - 1 \right) \times 100$$

the elongation Y (percent) in the second stretching bath is:

$$Y(\text{percent}) = \left( \frac{c}{b} - 1 \right) \times 100$$

and the total elongation Z (percent) is:

$$Z = \left( \frac{c}{a} - 1 \right) \times 100$$

Therefore, a relational formula can be obtained:

$$Z = X + Y + \frac{XY}{100}$$

Thus, the following conclusions can be obtained.

10 The maximum value obtainable by Z is dependent on the composition, viscosity and ripening degree of raw material viscose and compositions of the spinning bath and stretching bath, and further partition of the elongation in the first and second stretching baths. The first stretching bath comprising from 10 to 50 gm./liter.  $\text{H}_2\text{SO}_4$  and from 30 to 100 gm./liter  $\text{Na}_2\text{SO}_4$  is used below 50° C. and the second stretching bath comprising  $\text{Na}_2\text{SO}_4$  and  $\text{H}_2\text{SO}_4$  is used above 70° C. When each spun yarn is stretched respectively in the first and second stretching baths as strong as possible within a limit where no local breakage of threads occur, Z will reach to the maximum. It is evident that the excellent fiber can then be obtained.

15 Furthermore, in the relationship among elongations, X, Y and Z in each bath, if  $X/Z$  exceeds 3/4, the breakage of threads will become noticeable in the second bath and no smooth spinning can not be expected, while if  $X/Z$  is as low as below 1/4, the effect of elongation will not be sufficient as obvious in the following.

20 The relation between X and Z as just referred to has been ascertained to be applicable when a plurality of stretching baths are used.

25 The results obtainable due to varying stretching conditions referred to above for the spinning of yarn are shown in Table 2 in connection with embodiments of this invention, as follows: These data compare each result with the spinning solution and spinning conditions being held the same.

TABLE 2

|                       | a    | b    | c    | d    | e    | f    |
|-----------------------|------|------|------|------|------|------|
| Denier                | 1.3  | 1.3  | 1.3  | 1.3  | 1.3  | 1.3  |
| Strength (gm./d.)     |      |      |      |      |      |      |
| dry                   | 5.40 | 4.81 | 4.55 | 4.35 | 4.15 | 4.68 |
| wet                   | 4.12 | 3.80 | 3.21 | 3.18 | 2.86 | 3.68 |
| Knot                  | 1.65 | 1.38 | 1.34 | 1.46 | 1.58 | 1.48 |
| Elongation (percent): |      |      |      |      |      |      |
| dry                   | 5.9  | 5.6  | 5.8  | 6.5  | 7.9  | 6.2  |
| wet                   | 6.1  | 5.8  | 6.0  | 6.8  | 8.2  | 6.5  |
| Swelling degree       | 1.60 | 1.63 | 1.68 | 1.71 | 1.78 | 1.68 |

30 \* The process of the present invention.

35 <sup>b</sup> Hot weak acidic water baths are used at above 90° C. for the second and third baths; in the second bath, the maximum tolerance of elongation within which no local breakage of threads occurs is 180%. In this case, stretching could not be effected in the third bath and the reeling was carried out around the final spool at the velocity of 35 m./min. after passing same through the third bath.

40 <sup>c</sup> Water bath was used for the second bath at 30° C.; and when the third bath used was the same as (a), the elongation was 80% in the second bath, while the third bath allowed a tolerance of 50% maximum elongation to be effected.

45 <sup>d</sup> Both the second and third baths were used at 90° C.; 130% stretching was given in the second bath and the maximum tolerance of 15% stretching was given in the third bath.  $X/Z$  is 3.16/4.

50 <sup>e</sup> The second bath was set as (a), while the temperature of the third bath was 30° C. and stretching was given a maximum tolerance of 5% elongation.  $X/Z$  is 3.6/4.

55 <sup>f</sup> Both the second and third baths used were the same as described under (e); and when stretching was stopped at 50% in the second bath, 110% stretching was possible in the third bath. The total elongation Z is 215% and  $X/Z$  is 0.9/4.

60 Furthermore, according to the present invention, the lowering of strength of fibers due to alkaline water solution is less than that of the original fiber. For instance, the above-mentioned fibers (a) and (b) were immersed in 5% aqueous  $\text{NaOH}$  solution at 20° C. for 10 minutes without tension, thoroughly washed in dilute acetic acid and water and dried and then their strength was determined and the result was shown as percentages to the corresponding strength of the original sample as in Table 3. The fibers according to this invention show evidently

small lowering of strengths due to above-mentioned alkali treatment.

TABLE 3

| Specimens | dry strength, percent | wet strength, percent | knot strength, percent |
|-----------|-----------------------|-----------------------|------------------------|
| (a)-----  | 94.7                  | 95.0                  | 103.7                  |
| (b)-----  | 84.0                  | 86.1                  | 103.1                  |

## Example 1

Alkali which was prepared according to the ordinary way by steeping, pressing, and shredding from wood pulp, was aged for a short interval of time, then xanthated and dissolved in 50% by weight of cellulose of carbon bisulfide to produce viscose comprising 7% cellulose and 4.5% alkali content. Such viscose was then filtered and defoamed, when the temperature was kept as low as possible during the whole treatment from xanthation to spinning, and the viscose of 218 second viscosity and 15 salt index was spun into a spinning solution comprising 100 gm./liter  $\text{Na}_2\text{SO}_4$ , 65 gm./liter  $\text{H}_2\text{SO}_4$  and 5 gm./liter formaldehyde at 30° C. using a spinneret of 2000 holes of 0.065 mm. diameter. Said viscose was passed directly before spinning through a heat exchanger having a heat source of hot water and a pipe group secured between a curved spinning pipe and candle filter and the temperature of viscose was controlled to 60° C. at the outlet of the spinneret.

Such spun filaments were stretched to 230% in a slightly acidic second bath at 90° C., reeled, cut and purified in an ordinary process. The qualities of products thus obtained are shown under (e) of the following table.

When viscose was spun without heating in an entirely similar process, it was impossible to stretch above 120% in the second bath; and as a result, the resulting properties (c) were substantially the same as those spun similarly as (c) but without addition of formaldehyde as shown in table (a). On the other hand, the qualities obtained by proceeding the ageing of viscose to a salt index of 7 show remarkable degradation as shown in table (b).

As shown in (d) the properties of those spun in a similar process as that of (e) but without using formaldehyde were by far inferior to those obtained by the process under (e).

TABLE 4

| Process                                           | Comparision |             |             |             |                  |
|---------------------------------------------------|-------------|-------------|-------------|-------------|------------------|
|                                                   | (a) control | (b) control | (c) control | (d) control | (e) this process |
| Salt index of viscose-----                        | 15          | 7           | 15          | 15          | 15               |
| Formaldehyde in spin-bath (gm./liter)-----        | 0           | 5           | 5           | 0           | 5                |
| Spinnerette, viscose temperature (° C.)-----      | 15          | 60          | 15          | 60          | 60               |
| Denier-----                                       | 1.25        | 1.25        | 1.25        | 1.25        | 1.25             |
| Strength (gm./d.):                                |             |             |             |             |                  |
| dry-----                                          | 3.37        | 2.38        | 3.33        | 3.73        | 5.02             |
| wet-----                                          | 2.14        | 1.42        | 1.98        | 2.58        | 3.60             |
| knot-----                                         | 1.54        | 1.03        | 1.72        | 1.40        | 1.74             |
| Elongation (percent):                             |             |             |             |             |                  |
| dry-----                                          | 8.2         | 6.8         | 7.6         | 8.1         | 6.8              |
| wet-----                                          | 9.5         | 7.8         | 7.4         | 9.8         | 6.1              |
| Degree of swelling, percent-----                  | 84          | 115         | 85          | 73          | 61               |
| Load required for 5% wet elongation (gm./d.)----- | 0.96        | 0.42        | 0.75        | 0.90        | 2.85             |

Alkali cellulose, which was obtained by steeping and shedding from wood pulp in an ordinary process, was aged for a short interval of time and xanthated by using 38% carbon bisulfide of the weight of cellulose, then viscose was prepared to 8% cellulose and 5% alkali.

Such viscose was filtered and deaerated, with the operational temperature being held as low as possible from dissolving to spinning. The viscose of 108 second viscosity, 14 salt index was spun into a spinning bath comprising 90 gm./liter  $\text{Na}_2\text{SO}_4$ , 75 gm./liter  $\text{H}_2\text{SO}_4$ , 15

gm./liter  $\text{ZnSO}_4$  and 7 gm./liter formaldehyde at 32° C. through a spinneret having 4000 holes of 0.06 mm. diameter.

Said viscose was heated at 63° C. at the spinneret directly before spinning similarly as in Example 1.

The spun filaments were then passed through a slightly acidic second bath as 92° C. and stretched to 218% and reeled. Then, the resulting filaments were cut and purified as usual. The results are shown in table (c). Table (a) shows the results obtained by spinning in an entirely similar spinning bath excepting  $\text{Na}_2\text{SO}_4$  being 250 gm./liter and  $\text{H}_2\text{SO}_4$  95 gm./liter.

| 15                                                                | Method | (a) control | (b) control | (c) this invention |
|-------------------------------------------------------------------|--------|-------------|-------------|--------------------|
| Na <sub>2</sub> SO <sub>4</sub> (gm./liter) in spinning bath----- | 250    | 80          | 90          |                    |
| Viscose temperature at spinneret (° C.)-----                      | 63     | 19          | 63          |                    |
| Denier-----                                                       | 1.0    | 1.0         | 1.0         |                    |
| Strength (gm./d.):                                                |        |             |             |                    |
| conditioned-----                                                  | 3.38   | 3.92        | 5.05        |                    |
| wet-----                                                          | 2.26   | 2.36        | 3.64        |                    |
| knot-----                                                         | 1.41   | 1.65        | 1.67        |                    |
| Elongation (percent):                                             |        |             |             |                    |
| conditional-----                                                  | 7.3    | 6.8         | 5.4         |                    |
| wet-----                                                          | 9.2    | 7.2         | 5.4         |                    |
| Degree of swelling, percent-----                                  | 98     | 72          | 61          |                    |
| Load (gm./d.) required to produce 5% wet elongation-----          | 0.48   | 0.96        | 2.72        |                    |

## Example 3

Wood pulp was steeped, squeezed and shredded to obtain alkali cellulose. The resulting cellulose was aged in a short interval of time and xanthated using 40% carbon bisulfide based on the weight of cellulose used and further added 10% carbon bisulfide based on the weight of cellulose used at the beginning of xanthation. Such viscose contained 7% cellulose and 4.5% alkali, which was filtered and deaerated. The viscose was spun at viscosity 108 second and salt index of 18.2.

The spinning was performed at the operational temperature held as low as possible in a treatment from xanthation to spinning and in the spinning bath containing 65 gm./liter  $\text{H}_2\text{SO}_4$ , 95 gm./liter  $\text{Na}_2\text{SO}_4$  and 6 gm./liter formaldehyde at 28° C., through a 4000 hole spinneret of 0.06 mm. diameter.

Said viscose was heated immediately before spinning to 56° C. by passing through a heat exchanger secured between a gear pump and curved spinning pipe, of which heat source was hot water.

Spun filaments were passed through a second 2-meter bath containing 30 gm./liter  $\text{H}_2\text{SO}_4$  and 50 gm./liter  $\text{Na}_2\text{SO}_4$  at 30° C., while 130% stretching was given to the filaments. Further, said filaments were passed through a third bath of 1.5 meters, containing 60 gm./liter  $\text{H}_2\text{SO}_4$  and 100 gm./liter  $\text{Na}_2\text{SO}_4$  at 90° C., while the filaments were imparted 50% stretching.

In this case, the total stretching in the second and third baths are 245%.

The filaments were reeled around the final spool at a velocity of 35 m./min. and cut and purified by usual process. In this case, the properties of the filaments were as shown in Table 2.

What we claim is:

1. A process for manufacturing high tenacity viscose rayon filaments comprising heating to a temperature in the range of between 45° C. and 70° C. an unripened viscose having a salt index above 9 and having a viscosity ranging from 50 to 400 seconds, said viscose having an alkali content ranging from 0.5 to 0.9 times the cellulose content, then spinning said viscose in its heated state into an acid coagulating bath held at a temperature in the range of between a maximum of 35° C. and a minimum of below the viscose temperature by at least 20° C., said acid coagulating bath containing from 50 to 150 gm./liter  $\text{Na}_2\text{SO}_4$ , from 1 to 10 gm./liter formaldehyde, 30 gm./liter maximum  $\text{ZnSO}_4$  and 40 gm./liter minimum  $\text{H}_2\text{SO}_4$ .

2. The process as recited in claim 1, wherein spun filaments from said acid coagulating bath are stretched in a second bath at a temperature below 50° C. containing from 10 to 50 gm./liter  $H_2SO_4$  and from 30 to 100 gm./liter  $Na_2SO_4$ .

3. The process as recited in claim 2, wherein spun filaments from said second bath are stretched in a third bath at a temperature above 70° C. containing the same contents as said second bath and wherein the stretching of the spun filaments in said third bath ranges between one-fourth and three-fourths of the total stretching in both the second and third baths.

5  
10

4. The process as recited in claim 1 wherein the temperature to which said unripened viscose is heated is in the range of between 55° C. and 60° C.

References Cited in the file of this patent

UNITED STATES PATENTS

2,611,928 Merion et al. ----- Sept. 30, 1952  
2,705,184 Drisch et al. ----- Mar. 29, 1955  
2,937,070 Cox ----- May 17, 1960

FOREIGN PATENTS

854,152 Great Britain ----- Nov. 16, 1960